

Nov. 7, 1967

J. B. ULAM ET AL

3,350,772

METHODS OF CLADDING STAINLESS STEEL TO ALUMINUM

Filed Aug. 15, 1962



INVENTORS

John B. Ulam,  
William C. Camp

*Hooper, Leonard & Sull  
is a Attorney*

1

3,350,772

## METHODS OF CLADDING STAINLESS STEEL TO ALUMINUM

John B. Ulam and William C. Camp, Canonsburg, Pa., assignors to Composite Metal Products, Inc., a corporation of Pennsylvania

Filed Aug. 15, 1962, Ser. No. 217,036  
3 Claims. (Cl. 29—488)

This invention relates to methods of cladding metals and particularly to methods of bonding stainless steel to aluminum or other dissimilar metals together. Various methods of cladding metals have been heretofore proposed, however, these methods do have certain limitations and drawbacks. There are instances where it is desirable to have varying degrees of hardness in the two metals which form the composite clad or to control the physical properties of the two metals in the final product. This has been virtually impossible to accomplish in the methods heretofore proposed.

We have discovered a method of cladding metals which overcomes the difficulties of prior art practices and makes it possible to provide close control over the physical properties of the metals in the ultimate composite clad metal and at the same time to control and provide a strong bond between the dissimilar metals forming the clad body.

In the preferred practice of our invention, we clean the surfaces of the metals to be bonded by a mechanical or chemical procedure that removes all of the oxide from the surface. Preferably, the oxides, dirt, oil, etc., are removed by mechanical cleaning such as abrasive grinding so as to expose a perfectly clean surface. This practice is described in the Ulam Patents, 2,718,690 and 2,758,368. After the metals to be joined are cleaned they are heated in separate furnaces to a temperature selected to provide the desired characteristics in the finished metal and in an atmosphere which protects the metal surfaces from oxidation and the clean surfaces are then brought together within a like protective atmosphere and pressure is applied to cause the metals to be bonded and reduced. Preferably, the heating and bringing together of the clean surfaces is carried out in an inert atmosphere, a reducing atmosphere, or a vacuum.

In the accompanying figure, we have illustrated the practice of our invention as applied to a stainless clad aluminum.

In the figure, a coil of stainless steel 10 and a coil of aluminum 11 are fed on separate strip lines 13 and 14 to abrasive grinding wheels 15 and 16 which clean the two surfaces to be joined. The two strips are immediately carried into two separate heating chambers 17 and 18 which are provided with an inert gaseous atmosphere. In each of these furnaces 17 and 18, the strips of stainless and aluminum, respectively, are heated to temperatures above their stress relieving temperature, which temperatures are considerably different for these two metals. In the case of stainless steel in this example, the minimum temperature would be about 700° F. and the strip could

2

be heated as high as 1850° F. where full softening takes place. In the case of aluminum, the temperature would be about 465° F. The two strips are then brought together in a chamber 19 having the same inert atmosphere as the furnace while maintaining a temperature differential between them proportional to the difference of their minimum stress relieving temperatures. The strips are brought together by pinch rolls 20 and are fed into a rolling stand 21 where they are reduced and the bonding is completed.

By this practice, it is possible to heat the two metals to different temperatures, thus making possible fusion bonds, diffusion bonds or a combination of fusion and diffusion bonds. For example, if a cleaned stainless steel strip or sheet is led through furnace 17 which heats the stainless steel above its recrystallization temperature, as described above, and the aluminum is also heated in separate furnace 18 to a temperature above the recrystallization temperature and the two are rolled, there will result a fusion bond with both the stainless steel and the aluminum in the final clad product being in the fully annealed condition. Thus practice also permits more drastic reductions in the metals and thus stronger bonds. In this example, a 60% reduction in either the aluminum or the stainless above their recrystallization temperature has no effect on their ultimate ductility. A 60% reduction in stainless below its recrystallization temperature would be equivalent to 60% cold work and the resulting product would be useless in a forming operation.

In another example the stainless is heated above the recrystallization temperature and the aluminum below its recrystallization temperature. This would result in a combination fusion-diffusion bond with the stainless steel in the fully annealed condition and the aluminum partially hardened.

Another example would be the case where the stainless is heated to a temperature below the recrystallization temperature but above the minimum stress relieving temperature and the aluminum above its recrystallization temperature. This would result in a diffusion bond with fully annealed aluminum and partially hard stainless.

Still another example would require that the stainless be heated above the stress relieving temperature and the aluminum would be held at room temperature. This would result in a diffusion bond with stress relieved or fully annealed stainless steel and partially hardened aluminum.

It is obvious that a double stainless clad aluminum could be obtained by passing a second strip of stainless through a third furnace and bringing all three elements together with the aluminum as the core in a housing in an inert atmosphere similar to that described above.

Various degrees of hardness in both of the metals forming the composite can be attained by controlling the furnace temperatures and the final working of the strips in the formation of the clad metal. The varying physical properties which are thus attained can only be achieved by the practice of the present invention.

Typical mechanical properties that can be attained by the practice of this invention are shown in the accompanying table.

## TYPICAL MECHANICAL PROPERTIES

| Composite        |              |          |              | Gage | Yield Strength, p.s.i. | Tensile Strength, p.s.i. | Elongation in 2 in., percent |
|------------------|--------------|----------|--------------|------|------------------------|--------------------------|------------------------------|
| Stainless Steel  | Temp. (° F.) | Aluminum | Temp. (° F.) |      |                        |                          |                              |
| 304              | 975          | 3003     | 675          | .250 | 14,300                 | 18,900                   | 23                           |
| 304              | 1,100        | 3003     | 875          | .160 | 15,100                 | 21,100                   | 25                           |
| 304              | 900          | 3003     | 90           | .126 | <sup>1</sup> NT        | 21,700                   | 22.5                         |
| 304              | 1,600        | 3003     | 775          | .125 | 16,200                 | 21,200                   | 26                           |
| 304              | 1,250        | 3003     | 430          | .125 | <sup>1</sup> NT        | 21,500                   | 21.5                         |
| 304              | 1,465        | 3003     | 900          | .120 | <sup>1</sup> NT        | 22,000                   | 26.5                         |
| 304              | 950          | 1100     | 475          | .108 | 17,800                 | 23,600                   | 24                           |
| 304              | 1,700        | 3003     | 850          | .100 | 18,750                 | 23,800                   | 32.5                         |
| 304              | 1,625        | 1100     | 850          | .100 | 16,600                 | 22,100                   | 32.5                         |
| 304              | 1,325        | 3003     | 750          | .098 | 19,100                 | 24,900                   | 27                           |
| <sup>2</sup> 305 | 900          | 3003     | 700          | .097 | 19,200                 | 24,100                   | 21                           |
| 430              | 900          | 3003     | 250          | .095 | 23,110                 | 37,570                   | 18                           |
| 305              | 1,650        | 3003     | 750          | .094 | 19,800                 | 25,000                   | 26                           |
| 304              | 1,175        | 3003     | 575          | .091 | 23,760                 | 34,000                   | 18                           |
| 304              | 1,500        | 3003     | 750          | .091 | 24,350                 | 35,700                   | 22                           |
| 304              | 1,200        | 3003     | 850          | .090 | 21,300                 | 26,500                   | 25                           |
| 304              | 1,650        | 3003     | 800          | .077 | 21,500                 | 28,600                   | 30                           |
| 304              | 1,650        | 3003     | 850          | .075 | 23,300                 | 31,400                   | 34.5                         |
| 304              | 1,330        | 3003     | 700          | .067 | <sup>1</sup> NT        | 22,000                   | 24                           |
| 304              | 1,275        | 3003     | 700          | .066 | <sup>1</sup> NT        | 23,000                   | 26                           |
| 304              | 1,450        | 3003     | 700          | .052 | 24,750                 | 32,900                   | 27                           |
| 304              | 1,500        | 3003     | 750          | .052 | 26,700                 | 31,400                   | 28                           |
| 304              | 1,325        | 3003     | 650          | .050 | 24,600                 | 32,750                   | 28.5                         |
| 304              | 1,400        | 1100     | 890          | .050 | 18,210                 | 25,200                   | 27                           |
| 304              | 1,275        | 3003     | 775          | .046 | <sup>1</sup> NT        | 26,500                   | 23                           |
| 304              | 1,275        | 3003     | 775          | .043 | <sup>1</sup> NT        | 28,600                   | 23                           |
| <sup>2</sup> 304 | 1,175        | 3003     | 90           | .043 | <sup>1</sup> NT        | 29,100                   | 19                           |
| 304              | 990          | 3003     | 90           | .042 | <sup>1</sup> NT        | 28,700                   | 18                           |

<sup>1</sup> Not Taken. <sup>2</sup> Double Armor.

In the foregoing specification, we have illustrated certain preferred practices of our invention. It will be understood, however, that this invention may be otherwise practiced within the scope of the following claims.

We claim:

1. A method of forming a composite stainless steel and aluminum metal of at least one strip of each of aluminum and stainless steel comprising the steps of heating the strip of stainless steel above its stress relieving temperature but below its fusion temperature while maintaining the aluminum stress relieving temperatures, immediately bringing the surfaces of the heated stainless steel and the aluminum together and exerting pressure on the metals simultaneously to effect reduction and to form a bond between them.

2. A method of forming a composite stainless steel and aluminum metal of at least one strip of each of aluminum and stainless steel comprising the steps of separately and differentially heating each of the stainless steel and aluminum to a temperature above its own individual recrystallization temperature but below its fusion point and immediately bringing the differentially heated strips together while maintaining a temperature differential between them proportional to the difference of their minimum stress relieving temperatures and exerting pressure on the metals simultaneously to reduce and bond them.

3. A method of forming a composite stainless steel and aluminum metal of at least one strip of each of aluminum and stainless steel comprising the steps of separately and differentially heating each of the stainless steel and aluminum to a temperature above its own individual recrystallization temperature but below its fusion point, immediately bringing the differentially heated strips together while maintaining a temperature differential between them proportional to the difference of their minimum stress relieving temperatures and simultaneously reducing said sheets under pressure to produce at least a 60% reduction in the aluminum sheet.

## References Cited

## UNITED STATES PATENTS

|    |           |         |                       |            |
|----|-----------|---------|-----------------------|------------|
| 45 | 2,879,587 | 3/1959  | Mushovic et al. _____ | 29—504 X   |
|    | 2,908,073 | 10/1959 | Dulin _____           | 29—196.2 X |
|    | 3,078,563 | 2/1963  | Gould et al. _____    | 29—497.5 X |
|    | 3,095,500 | 6/1963  | Jost _____            | 29—497.5 X |
|    | 3,210,840 | 10/1965 | Ulam _____            | 29—488     |

JOHN F. CAMPBELL, Primary Examiner.

RICHARD M. WOOD, Examiner.

R. F. DROPKIN, Assistant Examiner.

UNITED STATES PATENT OFFICE  
CERTIFICATE OF CORRECTION

Patent No. 3,350,772

November 7, 1967

John B. Ulam et al.

It is hereby certified that error appears in the above numbered patent requiring correction and that the said Letters Patent should read as corrected below.

Column 2, line 22, for "Thus" read -- This --; column 3, in the table, first column, line 4 thereof, for "304" read -- 302 --; line 40, after "aluminum" insert -- below its --; same line 40, for "temperatures" read -- temperature --.

Signed and sealed this 7th day of January 1969.

(SEAL)

Attest:

Edward M. Fletcher, Jr.

Attesting Officer

EDWARD J. BRENNER

Commissioner of Patents